

## UNITED STATES PATENT OFFICE

1,973,119

## MANUFACTURE OF LUBRICATING OIL

Carey Forbes Spencer, Houston, Tex., assignor to  
Sinclair Refining Company, New York, N. Y., a  
corporation of Maine

No Drawing. Application March 9, 1932,  
Serial No. 597,799

4 Claims. (Cl. 196—1)

This invention relates to improvements in the manufacture of petroleum lubricating oils. More particularly, the invention relates to improvements in control of the color and the bloom of petroleum lubricating oils.

The color, by transmitted light, and the bloom, by reflected light, of petroleum lubricating oils are dependent not only upon the character of the crude petroleum from which the lubricating oil is derived but also upon the processing by which the lubricating oil is derived. The market, however, has tended to associate particular colors and blooms with particular characteristics. This tendency has imposed an added burden on the petroleum refiner in that it has subjected him to the necessity of controlling operations to produce lubricating oils of particular color and bloom as well as to produce lubricating oils having the required characteristics as lubricants. For example, a distilled lubricating oil and a residual lubricating oil having the same general characteristics may be derived from the same crude by different operations, the distilled product may be superior as a lubricant to the residual product, yet the distilled product may have a blue bloom whereas the residual product may have the green bloom required by the market for this particular product. This invention provides an improved control of the color and bloom of lubricating oils which is independent of the process by which the lubricating oil is produced.

In one aspect, this invention provides a method of imparting the required color and bloom to lubricating oils by means of a dye. In this aspect the invention provides a dye which imparts the required color and bloom to the lubricating oil when used in small proportions and which, within the range of proportions necessary to secure the required color and bloom, does not impair the properties of the petroleum lubricating oil with respect to emulsification or the stability of the oil, either during prolonged storage or during prolonged use, with respect to emulsification properties.

According to the present invention, a residual tar produced by the cracking of petroleum stock at temperatures upwards of 775° F. is subjected to treatment with sulphuric acid and the sludge formed as a consequence of this treatment is then separated from the tar, the acid treated tar is then neutralized with an aqueous solution of sodium carbonate and the resulting aqueous solution is separated from the tar, any low boiling hydrocarbons present are then distilled from the acid treated and neutralized tar under conditions

avoiding any substantial decomposition, and the residuum from this distillation is then blended with the petroleum lubricating oil in proportion not exceeding about 3% by volume on the lubricating oil. Percentages approximating 1—1.5% are usually sufficient to impart the required color and bloom to the lubricating oil. The residual tars produced by the cracking of petroleum stocks for the production of gasoline, by pressure distillation for example, are particularly useful in carrying out the invention. With the usual residual tars, the use of about 35—40 pounds of 95—100% sulphuric acid per barrel of the residual tar is advantageous. The neutralization is, with advantage, carried out at a temperature approximating 150—200° F. The residuum from the distillation may, with advantage, be filtered, through an absorbent earth for example, before blending with the lubricating oil.

The invention will be further illustrated by the following specific example of one operation embodying the invention: A residual tar having a gravity of 10—16° A. P. I., produced in the pressure distillation of Mid-Continent gas oil at a temperature of 800—850° F. for the production of gasoline, is agitated with 5—10 pounds of 98% sulphuric acid per barrel of tar at a temperature of 110—130° F. for 5—10 minutes by air blowing. After settling for 2—6 hours, the separated sludge is withdrawn. The tar is then agitated with 30 pounds of 98% sulphuric acid per barrel of tar at the same temperature by air blowing. The blowing is continued until a good separation, or "break", of the sludge formed is obtained without the addition of water. After settling for 2—6 hours the separated sludge is withdrawn. The tar is then blown with air for about 2 hours, or until free from sulphur dioxide, any separated sludge is withdrawn and after settling for 4—5 hours any further separated sludge is withdrawn. This acid treatment is carried out in the conventional agitator. Following the acid treatment, the tar is transferred to a so-called "wash tank" in which it is neutralized with 8—12% by volume of a 5—10° Bé. aqueous solution of soda ash, the temperature of the mixture being brought to 170—180° F. and held until a separation, or "break" of the solution is obtained. From 15—30 hours is usually required. The aqueous solution is withdrawn and the acid-treated and neutralized tar is washed with hot water until it tests free of alkali when boiled with distilled water, phenolphthalein being used as the indicator. The acid-treated and neutralized tar is then blown with air at a temperature of 170—180° F. until dry. It is then

transferred to a fire still and reduced with the use of sufficient steam to limit the maximum still temperature to about 500° F. to eliminate low boiling constituents. The residuum may have, 5 for example, a dark green color, a flash point of 380-430° F., and a viscosity approximating 1000 at 100° F. (Saybolt Universal). This residuum may be finished by filtration through 16-30 mesh Olmstead earth. This residuum product is the 10 dye of the invention. It is blended with lubricating oils, including distilled lubricating oils, in proportions up to about 3% by volume on lubricating oil. The volume of dye produced in carrying out the invention in this manner may approximate, 15 for example, 30-35% by volume on the residual tar subjected to treatment.

The invention is of special value and application in the manufacture of distilled petroleum lubricating oil. For example, the invention enables the conversion of distilled pale oils having a blue bloom to red oils having a green bloom. The invention is, however, of general application in control of color and bloom of lubricating oils, 20 enabling the petroleum refiner to control the manufacture of lubricating oils to produce lubricating oils having required characteristics as lubricants and independently to control this manufacture to produce lubricating oils having required color and bloom.

30 I claim:

1. In the manufacture of petroleum lubricating oils, the improvement which comprises subjecting a residual tar produced by the cracking of a petroleum stock at temperatures upwards of 775° F. 35 to treatment with sulphuric acid and thereafter separating the sludge formed, neutralizing the acid treated tar after sludge separation with an aqueous solution of sodium carbonate and thereafter separating the aqueous solution, distilling any low boiling hydrocarbons from the acid treated and neutralized tar under conditions avoiding any substantial decomposition, and thereafter blending the residuum with a lubricating oil in proportion not exceeding about 3% by volume on the lubricating oil, thereby imparting a green bloom to the lubricating oil.

2. In the manufacture of petroleum lubricating oils, the improvement which comprises subjecting a residual tar produced by the cracking of a petroleum stock at temperatures upwards of 775° F. 40

to treatment with sulphuric acid and thereafter separating the sludge formed, neutralizing the acid treated tar after sludge separation with an aqueous solution of sodium carbonate and thereafter separating the aqueous solution, distilling any low boiling hydrocarbons from the acid treated and neutralized tar under conditions avoiding any substantial decomposition, filtering the residuum with a lubricating oil in proportion not exceeding about 3% by volume on the lubricating oil, thereby imparting a green bloom to the lubricating oil.

3. In the manufacture of distilled petroleum lubricating oils, the improvement which comprises subjecting a residual tar produced by the cracking of petroleum stock at temperatures upwards of 775° F. to treatment with sulphuric acid and thereafter separating the sludge formed, neutralizing the acid treated tar after sludge separation with an aqueous solution of sodium carbonate and thereafter separating the aqueous solution, distilling any low boiling hydrocarbons from the acid treated and neutralized tar under conditions avoiding any substantial decomposition, and thereafter blending the residuum with a distilled lubricating oil in proportion not exceeding about 3% by volume on the lubricating oil, thereby imparting a green bloom to the lubricating oil.

4. In the manufacture of petroleum lubricating oils, the improvement which comprises subjecting a residual tar produced by the cracking of a petroleum stock at temperatures upwards of 775° F. to treatment with about 35-40 pounds of 95-100% sulphuric acid per barrel of the residual tar and thereafter separating the sludge formed, neutralizing the acid treated tar after sludge separation with an aqueous solution of sodium carbonate at a temperature approximating 150-200° F. and thereafter separating the aqueous solution, distilling any low boiling hydrocarbons from the acid treated and neutralized tar under conditions avoiding any substantial decomposition, and thereafter blending the residuum with a lubricating oil in proportion not exceeding about 3% by volume on the lubricating oil, thereby imparting a green bloom to the lubricating oil.

CAREY FORBES SPENCER.

125

55

130

60

135

65

140

70

145

75

150